

# UNITED STATES PATENT OFFICE.

FRANK F. HANSEN, OF CHICAGO, ILLINOIS, ASSIGNOR TO HANSEN-HALLIBURTON  
MFG. COMPANY, OF CHICAGO, ILLINOIS.

## ELECTRICAL-RESISTANCE ALLOY.

1,375,454.

Specification of Letters Patent. Patented Apr. 19, 1921.

No Drawing.

Application filed September 19, 1919. Serial No. 324,983.

To all whom it may concern:

Be it known that I, FRANK F. HANSEN, a citizen of the United States, residing at Chicago, in the county of Cook and State 5 of Illinois, have invented a certain new and useful Improvement in Electrical-Resistance Alloys, of which the following is a full, clear, concise, and exact description.

This invention relates to improvements in 10 electrical resistance alloys.

The invention is an improvement in those alloys such as used for electrical heating resistance units in flat irons, electric stoves, toasters, etc., and the object of the invention 15 is to provide such a resistance which will be comparatively inexpensive to manufacture, which will have a high fusing point, which will have long life, and which will have all the qualities desirable in an alloy required 20 to be drawn, and bent for commercial purposes.

In carrying out my invention, I combine 25 chromium, copper, tungsten and molybdenum. The chromium and copper are employed in a preponderating quantity because of their relative cheapness and conductivity and the tungsten and molybdenum are used in comparatively small quantities with the amount of tungsten somewhat exceeding the 30 amount of molybdenum.

I have found that the alloy may be made containing the elements within the limits indicated:

|             |            |
|-------------|------------|
| 35 Chromium | 30% to 60% |
| Copper      | 30% to 60% |
| Tungsten    | 2% to 5%   |
| Molybdenum  | 1% to 3%   |

The factors of cost, fusing point, conductivity, length of life, etc., taken into consideration, I have found that the following

approximate percentages give the greatest efficiency:

|            |     |    |
|------------|-----|----|
| Copper     | 50% | 45 |
| Chromium   | 45% |    |
| Tungsten   | 3%  |    |
| Molybdenum | 2%  |    |

An alloy of the composition hereinbefore indicated has a high fusing point approximately 50 1200° centigrade, can be easily and relatively inexpensively manufactured and is well adapted for drawing into wire as required for use in electrical heating units.

I claim:

1. An electrical resistance alloy containing principally chromium and copper in approximately equal amounts and small amounts of tungsten and molybdenum, the combined amount of tungsten and molybdenum being less than 10% with the tungsten in excess of the molybdenum. 60

2. An electrical resistance alloy containing, chromium 30% to 60%; copper 30% to 60%; and less than 10% of tungsten and 65 molybdenum combined, the tungsten being in excess of the molybdenum.

3. An electrical resistance alloy containing, chromium from 30% to 60%, copper from 30% to 60%, tungsten from 2% to 5%, 70 molybdenum from 1% to 3%.

4. An electrical resistance alloy containing, copper approximately 50%, chromium approximately 45%, tungsten approximately 3%, molybdenum approximately 2%. 75

In witness that I claim the foregoing I have hereunto subscribed my name this 2d day of Sept., 1919.

FRANK F. HANSEN.

Witness:

META SCHMIDT.